

## UNITED STATES PATENT OFFICE

2,571,688

## PRODUCTION OF COLLOIDAL SILVER

Harold Owen Dickinson, Ilford, England, assignor  
to Ilford Limited, Ilford, England, a British  
company

No Drawing. Application November 19, 1947, Se-  
rial No. 787,025. In Great Britain November  
29, 1946

2 Claims. (Cl. 252—313)

1

This invention relates to the production of colloidal silver and to the use of layers of such colloidal silver in colloid media in photographic materials.

It has long been known that by the addition of a reducing agent to a dispersion of a soluble silver salt in a colloid medium such as gelatin, there is slowly formed a colloidal dispersion of silver which is, in most cases, yellow in colour. Thus, one method which has been proposed is to add to a dispersion of silver nitrate in gelatin a quantity of hydrazine sulphate. The hydrazine sulphate is slowly added over a period of one hour and the resulting mixture allowed to stand at a slightly elevated temperature for a further three-quarters of an hour. In this way a yellow dispersion of colloidal silver is obtained.

Yellow colloidal silver thus formed is of value in photography as a medium for filter and anti-halation layers and various processes employing yellow colloidal silver for these purposes have been described in the literature.

The present invention is concerned with the production of colloidal silver which may be employed in the production of filter and anti-halation layers in photographic materials, and is based on the discovery that if there is present during the reaction a small proportion of silver sulphide or silver selenide nuclei, i. e. colloidal silver sulphide or silver selenide, the reaction proceeds at a very much accelerated rate, and yellow colloidal silver of excellent quality is obtained.

According to the present invention, therefore, colloidal silver is obtained by reacting in an aqueous colloidal medium a soluble salt of silver and a reducing agent therefor, in the presence of dispersed colloidal silver sulphide or silver selenide.

Whilst the process can be carried out in any water-permeable colloidal medium, e. g. an aqueous dispersion of polyvinyl alcohol or similar substance, it is preferred to effect the reaction in a gelatin medium. The silver salt employed may be any silver salt which is soluble in water and relatively easily reduced; silver nitrate appears to be particularly suitable. Whilst any reducing agent may be employed, it is preferred to use a reducing agent which is a good photographic developer, e. g. hydroquinone, p-hydroxyphenyl-amino-acetic acid, p-methyl-amino-phenol-sulphate, 1-phenyl-pyrazolidone-3, p-phenylenediamine and substitution derivatives. Relatively inefficient photographic developers, such as hydrazine, are less satisfactory. Particularly good results have been obtained with p-hydroxyphenylamino acetic acid.

2

The colloidal silver sulphide may be obtained quite readily by reaction between thiourea and silver nitrate. The preferred technique is to form the colloidal silver sulphide in the colloidal medium as a first step and then to add the soluble silver salt, and finally the reducing agent. The resulting dispersion containing colloidal silver may then be set, shredded, washed and re-dispersed in water, forming a coating solution from which filter and anti-halation layers of intense yellow colour and excellent quality may be obtained.

Colloidal silver selenide nuclei may be prepared by a precisely similar technique using selenourea instead of thiourea.

The quantities of the reagents and of the silver sulphide or selenide (which appears to act as a catalyst) may be varied widely, but the optimum quantity of silver nitrate appears to be of the order of 2 cc. of normal silver nitrate solution per 100 cc. of 5% gelatin solution. Smaller quantities than this give a lesser intensity of colour, and quantities below half the above concentration give only faint colouration. Larger quantities tend to give a rather turbid product, and for this reason it is preferred not to use more than twice the above concentration. It may be said in general therefore that for most purposes the quantity of silver nitrate should be of the order of 1 to 4 cc. of normal silver nitrate solution per 100 cc. of 5% gelatin solution. The quantity of reducing agent employed should be substantially chemically equivalent to the silver salt in order to obtain the best results. The optimum quantity of silver sulphide or selenide varies with the other factors but, for example, using a 3.5% solution of gelatin the best quantity appears to be that formed by the addition of 1 cc. of M/20 thiourea or selenourea with 1 cc. of N/10 silver nitrate per 200 cc. of the gelatin solution. Smaller quantities than this tend to give a somewhat greyish product, while higher quantities, e. g. up to 5 cc. of each component, appear to make no further difference to the intensity of the yellow colouration obtained.

45 The following examples illustrate the invention:

## Example 1

2 litres of a 3.5% aqueous solution of gelatin 50 was prepared and to this was added 10 cc. of M/20 thiourea and 10 cc. of N/10 silver nitrate. The solution was then digested for 20 minutes at 125° F. and then cooled to 90° F. There was then added 40 cc. of normal silver nitrate solution 55 followed by 400 cc. of N/10 p-hydroxy phenyl

amino acetic acid dissolved in N/10 caustic soda. A strong yellow colouration was immediately formed. The gelatin solution was then precipitated with ethyl alcohol. It was then soaked for three 10-minute periods in changes of water, and finally re-dispersed in a litre of water. This product, coated as a filter layer in a multilayer photographic material intended for colour photography, was found to have very good filtering characteristics and to have very little effect on the speed of the photographic emulsions with which it was in contact.

*Example 2*

The procedure of Example 1 was followed using an M/20 solution of selenourea instead of thiourea. Precisely similar results were obtained.

What I claim is:

1. Process for the production of colloidal silver which comprises reacting in an aqueous gelatin solution silver nitrate in the proportion of  $\frac{1}{2}$  volume of a  $\frac{1}{10}$  normal solution with  $\frac{1}{2}$  volume of a  $\frac{1}{20}$  molar solution of a compound taken from the group consisting of thiourea and selenourea and adding the colloidal silver salt formed which is taken from the group consisting of col-

loidal silver sulfide and colloidal silver selenide to an aqueous gelatin solution containing a quantity of silver nitrate equivalent to 1 to 4 volumes of normal silver nitrate solution per 100 volumes of gelatin solution and admixing a chemically equivalent quantity of photographic developing agent.

2. A process as in claim 1 wherein said photographic developing agent is p-hydroxyphenyl amino acetic acid.

HAROLD OWEN DICKINSON.

REFERENCES CITED

The following references are of record in the file of this patent:

UNITED STATES PATENTS

| Number    | Name            | Date         |
|-----------|-----------------|--------------|
| 1,119,647 | Schwerin        | Dec. 1, 1914 |
| 1,574,944 | Sheppard        | Mar. 2, 1926 |
| 2,220,187 | Wilmanns et al. | Nov. 5, 1940 |
| 2,420,956 | Kremers et al.  | May 20, 1947 |

FOREIGN PATENTS

| Number  | Country       | Date          |
|---------|---------------|---------------|
| 511,800 | Great Britain | Aug. 24, 1939 |